

June 7, 1927.

1,631,604

T. ROBINSON

ROOFING ELEMENT

Filed Nov. 21, 1923

Fig. 1,

3



Fig. 2,

3



Fig. 4



Fig. 3,



Fig. 5



Fig. 6,

7



Fig. 7.



INVENTOR

Thomas Robinson

BY

Pennie, Davis, Harris & Edwards  
its ATTORNEYS

## UNITED STATES PATENT OFFICE.

THOMAS ROBINSON, OF BABYLON, NEW YORK, ASSIGNOR TO ANACONDA SALES COMPANY, A CORPORATION OF DELAWARE.

## ROOFING ELEMENT.

Application filed November 21, 1923. Serial No. 675,998.

This invention relates to roofing material and more specifically to a material which consists of a nonmetallic base provided with a protective metallic coating applied to the 5 surface thereof.

Roofing material of the type above generally referred to has many distinctive and advantageous features owing to the fact that by selecting a base of suitable material and 10 applying a thin coating of non-corrodible metal thereover in a manner presently to be described, the roofing, when laid in place in the usual way, has the appearance of ordinary metal roofing but is considerably 15 cheaper, is easier to lay, and does not transmit heat so rapidly. Roofings formed of various compositions such as felt, asbestos, paper and the like, impregnated with bituminous or other similar compositions have 20 been widely used as a substitute for the ordinary wooden shingles but such material is objectionable in some instances on account of its appearance and also such compositions frequently have a tendency to deteriorate 25 when exposed to the weather and their edges may warp or curl. This composition roofing, however, is relatively cheap and is laid rapidly and at a low expense.

Metallic roofing material consisting of 30 zinc or copper shingles, plates, and the like, has been used to some extent and this metallic roofing is advantageous in that it has a longer life than the composition roofing above described. Also, the elements do not 35 warp or curl, but the roofing is considerably more expensive and requires greater attention in its application to the roof than does the composition. It conducts heat rapidly, however, and the cost of installation 40 is therefore increased by reason of the necessity of employing added layers of sheathing beneath it.

I have found, however, that a composite roofing which embodies the advantages of 45 both of the types above mentioned, while avoiding their disadvantages, may be prepared by using a cork base and applying to the surface thereof a coating of finely divided metal such as copper or zinc. The 50 cork base may be made of granulated cork held together by a binder or else the particles may be united into a comparatively rigid body by subjecting them to pressure and heat under regulated conditions. This treatment 55 causes the particles to be bound together

by the essential oils and resins present in the cork which are caused to exude under the application of heat and pressure and the particles are thus bound together and may be molded into blanks of the desired shape 60 and thickness. Such a cork base is non-hygrosopic, water-proof, a good heat insulator, and is also fire-resistant. It is light in weight and may be readily nailed or cut by sawing. The metal coating of which I 65 prefer to make use is finely divided copper, which is applied to the surface of the cork base either dry or suspended in a binding vehicle. When the metal is used dry it is blown or sprayed upon the surface of the 70 cork which has been preliminarily treated with a suitable adhesive. For a binding vehicle in which the metal particles may be suspended I prefer to make use of nitrated cellulose and the suspension may be blown 75 or sprayed over the surface to be given the coating. A roofing element of this construction is satisfactory for many purposes but if desired for any reason to increase the thickness of the metal then the finely divided 80 particles may be used as a conducting coating over which a layer of copper may be electrodeposited.

Such roofing material as I have above described is capable of use for many purposes 85 and for commercial transportation it will be made in a number of standard forms, such as strips, boards, single and multiple unit shingles, Spanish and mission tiles, and the like.

In the accompanying drawings I have illustrated two commercial forms of roofing element constructed in accordance with this invention, and in these drawings,

Fig. 1 is a face view of such an element, 95  
Fig. 2 is an end view,

Fig. 3 is a cross-sectional view on the line 3—3 of Fig. 1,

Fig. 4 is a face view of a single shingle,

Fig. 5 is a fragmentary cross-sectional 100 view on a somewhat enlarged scale,

Fig. 6 is a face view of a portion of a roofing element having two coatings of metal, and

Fig. 7 is a cross-sectional view on the line 105 7—7 of Fig. 6.

In these drawings, the base of a three-unit shingle is represented by the reference character 8. This base is of rectangular form and will be seen to have cut-outs 9 on 110

one edge, these cut-outs being formed for the purpose of giving the element the appearance of three separate shingles when the multiple unit elements are laid in courses on the roof. The base is made of molded and compressed cork, either with or without a binder. If no binder is to be used, the granulated cork is pressed at a raised temperature so that the essential oils in the particles will serve as the binding ingredient. If a binding material is used, however, it will be of the type commonly used in connection with the manufacture of granulated cork slabs. The surface dimensions and thickness of the base will depend on the purpose for which it is to be used.

These bases, molded or otherwise formed to the proper size and shape, are next given a protective metallic coating and this coating is limited preferably, for reasons of economy, to that portion of the surface which is exposed when the elements are laid. In Fig. 1 there is shown a three-element shingle which has a pair of cut-outs 9 with the edges at the ends of the element also slightly recessed as at 10, so that when two elements are laid side by side a cut-out is formed in their abutting edges. When two courses have been laid in place the cut-outs in the overlying course will expose portions of the elements in the course next beneath. It is, therefore, necessary, in order that all portions of the base should be protected, to give the protective coating the somewhat irregular form illustrated in Fig. 1, the tongues 11, 11, extending from the main body of the coating so as to underlie the cut-outs of the shingles to be laid in the course next above and thus insure that all portions of the element which are exposed may be protected by a metal coating. It will be noted also that the edges of the element along the portion to be exposed are beveled as shown at 12, this bevel being so formed that the coating will cover the edges of the element completely.

The metallic coating 13 is made of powdered metal, preferably a non-corrodible metal, such as copper or zinc. This powdered metal may be blown or otherwise applied in a dry form to the surface of the base, a suitable adhesive having first been applied thereto, but I prefer to use for this purpose a suspension of the powdered material in a binding vehicle such as nitrated cellulose. This suspension may be easily applied to the surface of the base so as to give a uniform coating thereto, and it may be applied also in such a way as to cover only those portions of the base where it is required. As a specific example of the proportions of binding material and metal to be used, and also of the quantities required to apply a film of satisfactory thickness, the following is given by way of example:

A quantity of finely divided copper, ranging in weight from 3 to 7 pounds, is introduced into a gallon of a spraying solution, preferably nitrated cellulose. The solution is thoroughly agitated so as to make a uniform suspension of the copper in the liquid, and this liquid is then sprayed on the surface of the base, preferably in such proportions that between one and two ounces of metal are deposited upon each square foot of the material to be treated. The mixture of powdered copper and the binding vehicle will be applied to all portions of the base which are exposed when the latter is laid in position on the roof. The metal, therefore, will not only cover the weather surface, but will also cover the beveled portions of the edges of the element and also the tongues 11. After the powdered metal has been applied in the manner above described the element is allowed to dry until the binding vehicle sets and then the element may be used without further treatment, or else if desired, the metal may be given a surface treatment, as for instance by burnishing or by chemical treatment so as to alter the color of the metal. This latter method of treatment is particularly applicable when copper has been used as the protective metal. The coloring of the copper particles is carried on by various methods which are well-known and the copper may be given several different colors which may be desirable in the particular location where the material is to be employed.

The method of manufacturing the single unit shingle illustrated in Fig. 4 is similar to the method above described. This element is of a size corresponding substantially to that of the usual wood shingle and has a metal surface 14 applied over that portion of its face which will be exposed when the shingle is laid in place. The exposed edges of this portion of the shingle are beveled as indicated at 15, and also cut away at 16 so that when two shingles are laid side by side the rear portions 17 of their lateral margins will lie close together, while the cut-outs 16 of the adjacent shingles will cooperate to give the pair of shingles the appearance of being separated as is usual in a wooden shingled roof. The metal coating also has a rearwardly projecting tongue 18 which underlies the cut-out portions of a pair of shingles of the course next above.

In Fig. 5 the base 8 is shown in somewhat enlarged size and it will be noted that this base along the outer surface 19 has a somewhat irregular appearance, the fine irregularities occurring during the manufacture of the base. These irregularities would ordinarily be considered a detriment in a plain composition base but in the case of the composite roofing element under discussion the irregularities serve a useful purpose and no attempt is made to remove them from the 130

base surface. On the contrary, the application of the metal over these irregularities not only serves to give the metallic surface a slightly roughened appearance so that it 5 has a texture, but the particles of metal enter into the many small depressions in the surface of the base and are thus held firmly in place, the adherence of the binding vehicle being more satisfactory in the case of 10 a slightly roughened surface than is true in connection with a base which has been intentionally given a smooth surface.

While the roofing element which has been above described consisting of a base made of 15 cork and having a surface formed of metallic particles bound to the cork is satisfactory for many purposes, it may be desirable in some instances to apply a thicker coating of metal, and this may be readily 20 done by using the element above described as a cathode in an electrolytic tank and then depositing a further thickness of the metal electrolytically upon the powdered metal, this outer layer of metal applied by electro- 25 deposition consisting of a multiplicity of fine particles united molecularly to form a substantially continuous coating. For this purpose it is preferable to make use of a base upon the surface of which the powdered 30 metal has been applied in the dry form; that is, the base should first be treated with an adhesive and the powdered metal blown or otherwise distributed over the surface of the adhesive. With this treatment the copper 35 particles on the surface have exposed portions which are not covered by the adhesive. These surface particles form a conducting layer which may be connected with the negative terminal of an electrolytic cell which 40 contains an electrolyte consisting of a salt of the metal to be deposited. It is preferable, though not essential, to use the same metal in the outer coating that is used in the first application of the base, and the 45 metal electrodeposited will be plated upon the particles and thus the entire coating will be bound firmly to the surface of the base. Such an element is illustrated in Figs. 6 and 50 7 in which it will be seen that the first coating 13 conforms closely to the surface irregularities and that the outer coating 20 deposited thereover also has an irregular surface, although the lesser irregularities of the coating 13 are now somewhat smoothed off. 55 However, the outer layer still has the roughened appearance usually preferable to the smooth surface which is normally present in the case of plain sheet metal roofing.

While I have described the manufacture of the roofing as being carried on by the treatment of elements in the form in which they are finally to be used, it will be clear that it is possible to make use of standard sizes of base blanks, apply the metal to these blanks, and thereafter cut them to the desired shape 60 and form. Also it is not essential that the base should be formed as a flat slab but it may be given the curved formation of an English tile. In fact, it is possible to produce roofing elements in any of the various 65 irregular sizes and shapes, such as are commonly used at the present time.

The choice of metals that may be applied according to this invention is unrestricted 70 but the selection of the metal will depend on the purpose for which the roofing is to be employed, and will also depend on the cost of the finished product. In general, copper, zinc, aluminum, or various bronzes are the 75 metals which will have the widest application, and the weight of the metal will vary between one and two ounces per square foot, although this will depend on the ultimate use of the element and also on the kind of metal. For instance, if aluminum is employed a reduced weight of this material will 80 form a metallized surface of the desired thickness. In the preferred embodiment of the invention nitrated cellulose is employed 85 as the suspension medium, but many other materials such as drying oils, for example, 90 may also be made use of.

I claim:

1. A roofing element which comprises a substantially rigid body of compressed cork particles bound together by the adhesive resinous constituents thereof, and a layer of finely divided metallic particles adhesively affixed to the surface of the body. 95

2. A roofing element which comprises a substantially rigid body of compressed cork particles bound together by the adhesive resinous constituents thereof, a coating of an adhesive over the body, and a layer of finely divided metallic particles over the coating. 100

3. A roofing element which comprises a substantially rigid body of compressed cork particles bound together by the adhesive resinous constituents thereof, a coating of an adhesive over the body, a layer of finely divided metallic particles over the coating, and a substantially continuous layer of molecularly united metallic particles over the first layer. 110

In testimony whereof I affix my signature.  
THOMAS ROBINSON.